# EUROPEAN PATENT SPECIFICATION

(11) **EP 0 116 460 B1**
(45) Date of publication and mention of the grant of the patent: **12.08.1987**
(21) Application number: 84300788.1
(22) Date of filing: 08.02.1984
(51) Int. Cl.: C10M 135/12, C10N 40/08

(54) **Friction modifier additive for power transmission shift fluids**
Reibungsmodifizierender Zusatz für Kraftübertragungsflüssigkeiten
Additif modifiant la friction pour fluides de transmission d'énergie

(30) Priority: 08.02.1983 US 464950
(43) Date of publication of application: 22.08.1984
(73) Proprietor: EXXON RESEARCH AND ENGINEERING COMPANY, Florham Park, New Jersey 07932-0390 (US)
(72) Inventor: Gutierrez, Antonio, Mercerville New Jersey (US); O'Halloran, Rosemary, Union New Jersey (US); Brois, Stanley James, Westfield New Jersey (US)
(74) Representative: Bawden, Peter Charles

## Description

This invention relates to the use in power transmission shift fluids, such as automatic transmission fluids of an additive effective in providing friction modification benefits.

Mineral oil based power transmission shift fluids, or functional fluids, such as automatic transmission fluids are required to exhibit a number of properties such as antiwear, friction modification, oxidation inhibition, anticorrosion, demulsification and the like in order to qualify for commercial acceptance.

Prior art references pertinent to this invention include U.S. Patent 3,852,205, issued December 3, 1974 to Kablaoui et al., which discloses automatic transmission fluid containing either S-carboxy alkylene hydrocarbyl succinimide or hydrocarbylsuccinamic acid. These are prepared in a two-stage process comprising reacting maleic anhydride with a primary amine in a 1:1 mole ratio. The amine and imide product so formed is then contacted with a thiocarboxylic acid to form the desired additive. U.S. Patent 4,129,510, issued December 12,1978 to Smith, disclosed sulfur-containing additive derived from reacting a hydrocarbyl mercaptan having 1 to 5 SH groups with a C₃ to C₃₈ aldehyde or ketone to form an intermediate which is subsequently reacted with an olefinic carboxylic acid or functional derivative. The products are said to be useful as oxidation and rust inhibitors in lubricants and fuels.

In accordance with the present invention it has been discovered that additives being represented by the formula: wherein R' is an alkyl of about 8 to 30 carbon atoms and R is a lower Cₗ-C₄ alkyl or hydrogen are effective in modifying the friction properties of power transmission fluids. Preferred is the use of those compounds where the total R'(R)CHCH₂- group has about 16 to 20, such as 18, carbon atoms.

A particularly preferred embodiment of the present invention is the addition product of octadecyl mercaptan with maleic anhydride. Compounds of the invention may also be prepared by addition of mercapto diacids to terminal olefins, e.g., R'(R)C=CH₂.

The additives are generally used within the range of about 0.01 to 1 wt% to provide the effective friction properties. Preferably, the power transmission shift fluids will contain about 0.1 to 0.5 wt% of the additive of the present invention. Octadecyl thiosuccinic acid or anhydride are preferred additives of this invention.

In addition to use in automatic transmission fluids the additive of the present invention will function as a friction modifier in other power transmission shift fluids based on mineral oils such as hydraulic fluids, power brake and power steering fluids, heavy duty equipment fluids and the like.

Friction modification is one of the most demanding properties to effectively provide in an automatic transmission fluid and is considered the characteristic which distinguishes ATF compositions from other categories of lubricants. Very specific frictional properties related to transmission parts operation must be met in order to have an acceptable fluid. The additive of the present invention is highly advantageous in that it satisfies at low treat levels the significant friction modification tests, and is efficiently prepared at relatively lower costs thereby providing a more effective and economical automatic transmission fluid. The properties evaluated in ATF tests an specifications are generally applicable to other power shift transmission fluids.

Automatic transmission fluids containing the additive of the present invention are the preferred embodiment. Such ATF compositions contain a number of conventional additives in amounts providing their normal attendant functions and are typically blended into the mineral oil base in the following ranges:

Typical base oils for automatic tranmission fluids and power transmission shift fluids generally include a wide variety of light hydrocarbon mineral oils, such as naphthenic base, paraffin base and mixtures thereof, having a lubricating viscosity range of about 34 to 45 SUS (Saybolt Universal Seconds) at 38°C.

The invention is further illustrated by the following examples which are not to be considered as limitative of its scope. ATF compositions used in the examples below were formulated in accordance with the components and concentrations noted above (referred to as Base Fluid) except the friction modifier was the compound of this invention used in the amounts reported below.

### Example 1

About 100 g (0.35 moles) of octadecyl mercaptan were dissolved in 100 ml of tetrahydrofuran (THF). Then, about 34.2 g (0.35 moles) of maleic anhydride were added, followed by the addition of 1 ml of triethylamine as catalyst. The reaction mixture was heated to reflux for about one hour. At the end of the hour, the THF solution was poured into a large volume of pentane and a white solid precipitated out of solution. The white solid was filtered, and dried in vacuo until constant weight. The infrared spectrum of the solid revealed no unreacted maleic anhydride present. It analyzed for 68.85% C, 10.52% H and 8.77% S which is consistent with the desired alkylthio succinic anhydride that required 68.70% C, 10.48% H and 8.34% S.

### Example 2

About 30 g (0.2 mole) of mercapto-succinic acid were dissolved in 200 ml of methanol and cooled to about 15°C. Thereafter, 56 g (0.2 mole, 90%) of 1-octadecene were added, followed by the addition of 1.5 g of Lucidol 70 radical initiator (Benzoyl peroxide, 70%). The reaction mixture was rapidly stirred for about two hours, while some crystalline white solid formed. The reaction temperature rose to 30°C during the first half hour and then about 25°C for the rest of the reaction time. The white solid was filtered and collected. The infrared spectrum of the solid is consistent with the desired 2-(octadecylthio) succininic acid. The solid analyzed for 66.77% C, 1045% H, and 8.10% S. Theory requires 65.67% C, 10.52% H and 7.97% S.

### Example 3

To a formulated automatic transmission fluid (Base Fluid) was added 0.25 wt% of the octadecylthio succinic anhydride of Example 1 and the fluid was evaluated for its friction properties in the Davison Friction Test utilizing the SAE No. 2 Friction Machine; dynamic and static torque values were within the test specification of General Motor Dexrom^{O} II Automatic Transmission Fluid (GM specification G137-M, July, 1980). Torque values were measured at 3 phases: (1) 16,500 Ib-ft,. 1 sec. lock-up, (2) 7,200 Ib-ft, 40 Ib pressure and (3) 16,500 Ib ft, 60 Ib pressure. Phase 1 friction torque tracings showed results of 102, 91 and 84; phase 2 showed 101, 97 and 88 and phase 3 showed 138, 130 and 123 ft-Ibs.

## Claims

1. The use as an additive for modifying the friction of power transmission fluids of the formulas: wherein R' an alkyl of about 8 to 30 carbon atoms and R is a lower C₁-C₄ alkyl or hydrogen.

2. The use according to claim 1 of 0.01 to 1 wt% of said additive.

3. The use according to claim 1 or claim 2 wherein the fluid is an automatic transmission fluid.

4. The use according to any of the preceding claims wherein said additive is octadecyl thiosuccinic anhydride or acid present in an amount of about 0.1 to 0.5 wt%.

5. The use according to any of the preceding claims wherein R'(R)CHCH₂ groups has a total of about 16 to 20 carbon atoms.

## Patentansprüche

1. Verwendung von Verbindungen mit den Formeln: in denen R' ein Alkylrest mit etwa 8 bis 30 Kohlenstoffatomen und R ein niederer C₁-C₄-Alkylrest oder Wasserstoff sind, als.Additiv zum Modifizieren der Reibung von Kraftübertragungsfluiden.

2. Verwendung nach Anspruch 2, dadurch gekennzeichnet, daß man 0,01 bis 1 Gew.% des Additivs verwendet.

3. Verwendung nach Anspruch 1 oder 2, dadurch gekennzeichnet, daß das Fluid ein automatisches Getriebeöl ist.

4. Verwendung nach einem der vorangehenden Ansprüche, dadurch gekennzeichnet, daß das Additiv Octadecylthiobernsteinsäureanhydrid oder -säure ist und in einer Menge von etwa 0,1 bis 0,5 Gew.% vorhanden ist.

5. Verwendung nach einem der vorangehenden Ansprüche, dadurch gekennzeichnet, daß die R'(R)CHCH₂-Gruppe insgesamt etwa 16 bis 20 Kohlenstoffatome besitzt.

## Revendications

1. Utilisation comme additif pour modifier la friction de fluides de transmission de puissance, de composés de formules: où R' est un groupe alkyle ayant environ 8 à 30 atomes de carbone et R est un groupe alkyle inférieur en Ci à C₄ ou l'hydrogène.

2. Utilisation suivant la revendication 1 de 0,01 à 1% en poids dudit additif.

3. Utilisation suivant la revendication 1 ou la revendication 2, dans laquelle le fluide est un fluide de transmission automatique.

4. Utilisation suivant l'une quelconque des revendications précédentes, dans laquelle ledit additif est l'ahydride ou l'acide octadécylthiosuccinique en une quantité d'environ 0,1 à 0,5% en poids.

5. Utilisation suivant l'une quelconque des revendications précédentes, dans laquelle le groupe R'(R)CHCH₂ a un total d'environ 16 à 20 atomes de carbone.
